# EUROPEAN PATENT SPECIFICATION

(11) **EP 0 049 921 B1**
(45) Date of publication and mention of the grant of the patent: **06.02.1985**
(21) Application number: 81201092.4
(22) Date of filing: 02.10.1981
(51) Int. Cl.: C10L 1/32, C10L 1/02, C10L 1/18

(54) **Clear liquid fuel mixture for combustion engines**
Klares, flüssiges Kraftstoffgemisch für Verbrennungsmotoren
Mélange liquide de combustible liquide pour moteurs à combustion

(30) Priority: 09.10.1980 NL 8005581
(43) Date of publication of application: 21.04.1982
(73) Proprietor: STAMICARBON B.V., NL-6167 AC Geleen (NL)
(72) Inventor: Donners, Wilhelmus Aloisius Barbara, NL-6118 CN Nieuwstadt (NL); Hovestreydt, Gerrit, NL-6165 EA Geleen (NL); Den Otter, Marinus Johannes A. M., NL-6151 BH Munstergeleen (NL)
(74) Representative: Hoogstraten, Willem Cornelis Roeland

## Description

The invention relates to a clear liquid mixture for application as fuel in combustion engines, comprising:
a liquid hydrocarbon mixture;
water;
an alcohol fully soluble in water;
surface-active substances.
Such a clear, liquid fuel mixture is known from United States patent 4,002,435.

The fuel mixture described in this patent specification consists of:
a. petrol or diesel oil;
b. 0.1-10% of water;
c. 0.1-20% of an alcohol fully soluble in water and
d. a combination of surface-active agents, consisting of:
   1. a salt of saturated or unsaturated higher fatty acid;
   2. an unsaturated organic acid; and
   3. an ethylene oxide condensation product.

According to this patent specification, a special combination of surface-active agents is required for the dispersion of alcohol and water in petrol or oil in order to obtain a stable water-containing fuel mixture with a water-soluble alcohol, such as methanol. As alcohol fully soluble in water, methanol, ethanol, propanol or a mixture of these alcohols is applied.

The disadvantage of this fuel mixture is that it is relatively expensive, because special surface-active agents are necessary for dispersing the alcohols fully soluble in water in petrol to a mixture which is stable over a wide temperature range.

The Dutch patent application 7416290 relates to the operation of Otto and rotary piston engine, using petrol as fuel simultaneously with water-containing crude methanol. It is true that the alcohol used is cheap, but this is amply offset by the disadvantage that for each motor vehicle separate tanks and separate injection systems for the petrol and for the water-containing crude methanol are required. When combined in advance, such a mixture will show phase separation, which makes application impossible. In order to be able to use this fuel each motor vehicle, will require the necessary investments.

The European patent application 12345 relates to engine and turbine fuels containing water and alcohol and using a special and expensive nonionogenic emulsifier to obtain good stability, even in coldness. Relatively much stirring energy is required in order to prepare a milky emulsion of the various components. Another disadvantage is that, if this fuel mixture has been left to stand for some time, or if unfortunately water has found its way into it, further stirring energy will be required again in order to obtain an emulsion. This is rather problematical if this fuel mixture is contained in the tank of a motor vehicle. Furthermore, it is difficult to determine if phase separation has already taken place. The stability in coldness, too, is not quite satisfactory.

From FR-A-2114465 a one phase system of a combustion fuel is known which discloses a complex mixture of a fuel, purified methanol and further additives.

The purpose of the invention is to remove the said disadvantages and to provide a clear liquid fuel mixture for combustion engines, as stated in the preamble, which fuel mixture is cheap, does not separate out even after it has been left to stand for a long time, which is stable at -20°C and which allows the various components to be mixed with each other virtually without use of stirring energy to form a clear liquid mixture.

A further purpose of the invention is to provide a fuel mixture containing relatively few petroleum- recovered hydrocarbons and relatively many liquid raw materials which can be prepared from natural gas and/or coal. Furthermore, the fuel mixture must be applicable in the existing engines.

It has been found that higher alcohols not or sparingly soluble in water have a positive effect on the increase of the stability range of clear fuel mixtures containing hydrocarbons, methanol and water, even if these higher alcohols are present in very small quantities. Very small quantities are understood to mean quantities in the order of 0.02% by volume.

It is very important for the stability range, i.e. the range in which a clear mixture is obtained and/or kept, to be as wide as possible, particularly at -20°C. This will strongly reduce the risk of phase separation at fluctuations in the composition of the mixture. Furthermore, it will also give greater freedom in the composition of the fuel mixture.

According to the invention the fuel mixture consists of:
a. a liquid hydrocarbon mixture;
b. a mixture of methanol, water and higher alcohols, that has been obtained by steam reforming of methane and subsequent catalytic synthesis of the gas mixture obtained, in such amount that the fuel mixture contains 1-10% by weight of water; 0,1-25% by weight of methanol and 0,01-20% by weight of alcohols with 4 to 12 C atoms not or sparingly soluble in water;
c. 0.1-15% by weight of surface-active substances; and optionally
d. 5-20% by weight of an alcohol with 2-12 C atoms, and/or
e. 0,01-15% by weight of an ether with 2-8 C atoms.

The alcohols with 4-12 C atoms not or sparingly solubility in water may also be divalent alcohols, such as diols. Preference, however, is given to monovalent alcohols.

According to the invention it is possible to incorporate the mixture of methanol, water and higher alcohols in hydrocarbons just by means of surface-active substances, although it is an advantage to add optionally an extra quantity of alcohol with 2 to 12 C atoms, or with 2-8 C atoms, because the quantity of surface-active substances required may then be smaller. Optionally 5-20% by weight respectively 0,01-15% by weight of these alcohols may be added.

Sparingly soluble in water is understood here to mean that only very subordinate quantities will dissolve in water, i.e. smaller than 25% by weight, preferably smaller than 10% weight.

The mixture can be converted very simply into a clear whole. This can be done by shaking, filling of the storage tank or simply by transport.

The fuel mixture according to the invention has the following advantages:
a. it is clear;
b. requires little or no stirring energy during its preparation;
c. is stable to at least -20°C;
d. gives lower emission of harmful components in the exhaust gases than petrol;
e. gives good knock resistance so that the addition of tetra-alkyl lead to raise the octane number is not necessary.

It has specifically been found that, in addition to small quantities of these higher alcohols not or sparingly soluble in water, a larger quantity of alcohols with 2-4 C atoms fully soluble in water has the effect that a substantially smaller quantity of surface-active agents is required.

By the addition or use of larger quantities of alcohols with 4-12 C atoms not or sparingly soluble in water, the quantity of surface-active substances can be reduced, while a simultaneous widening of the stability range will be found.

Another major advantage of the invention is that, without adversely effecting the clearness and stability of the fuel mixture, the quantities of water-soluble alcohols and alcohols not or sparingly soluble in water can be varied in respect of each other.

Thus in the liquid mixture according to the invention methanol, water and higher alcohol may be present in such amounts that the fuel mixture contains 1-10% by weight of water; 0,1-25% by weight of methanol; 0,01-20% by weight of alcohols with 4 to 12 C atoms not or sparingly soluble in water and 5-10% by weight of alcohols with 2-4 C atoms fully soluble in water.

Another liquid mixture according to the invention may contain methanol, water and higher alcohols in such an amount that the fuel mixture contains 1-10 by weight of water, 0,1-25% by weight of methanol, 5-20% by weight of alcohols with 4-12 C atoms not or sparingly soluble in water and 0,01 -5% by weight of alcohols with 2-4 C atoms fully soluble in water.

The alcohol with 2-4 C atoms fully soluble in water is preferably tertiary butanol, together with the small quantities of alcohols not or sparingly soluble in water.

Preferably the alcohol with 4-12 C atoms not or sparingly soluble in water is n-butanol or n-pentanol.

As stated earlier, the quantities of water and methanol in the liquid mixture can be varied in respect of each other. In the liquid mixture according to the invention preferably methanol, water and higher alcohols are present in such amounts that the fuel mixture contains 1-5% by weight of water and 2-15% by weight of methanol.

For dispersing the water and the alcohols in the petrol, surface-active substances are required.

It is supposed that a so-called micro-emulsion is formed, which is understood to mean a transparent, stable, liquid system consisting of at least two liquids which cannot or hardly be mixed, in which system one liquid is dispersed by means of one or more surface-active substances in the other. The drop size is substantially smaller than that of an ordinary emulsion and, in consequence, a micro-emulsion, unlike an ordinary emulsion, is transparent. Apart from the limited amount of energy required for mixing the components, the formation of micro-emulsions requires no special measures. They are formed spontaneously as soon as the various components are brought together. Preferably anionogenic or nonionogenic surface-active substances and specifically combinations thereof are applied. A mixture of surface-active acid and salts of these acids as surface-active substances have the greatest preference, because these have been found very suitable and are, moreover, cheap. The liquid mixture preferably contains 0.1-10% by weight of surface-active substances. The quantity can easily be determined by one skilled in the art. If a nonclear emulsion is formed, the quantity must be increased.

As anionogenic surface-active substances the following are eligible:
- salts of surface-active carboxylic acids, specifically fatty acids with 10 to 20 C atoms;
- sulphuric acid esters, specifically alkyl esters with an alkyl group of 10 to 20 C atoms;
- alkyl and alkylaryl sulphonates, in which the alkyl group has 10 to 20 C atoms and the alkylaryl group 10 to 26 C atoms;
- paraffin sulphonates, lignin sulphonates;
- phosphoric acid esters, specifically alkyl esters with an alkyl group of 10 to 20 C atoms;
- salts of surface-active phosphorous and phosphoric acids.

As nonionogenic surface-active substances the following are eligible:
- ethylene oxide condensation products with, for instance, alcohols with 6 to 18 C atoms, alkyl phenols, polyols or propylene oxide;
- polyhydroxy compounds, such as esters of polyols and fatty acids;
- fatty acids, both saturated and unsaturated, with 10 to 20 C atoms.

It is a great advantage of the present invention that a mixture can directly be applied as obtained in the preparation of methanol, starting form methane, without water and higher alcohols having to be removed.

A mixture of methanol, water and alcohols not or sparingly soluble in water can be obtained directly by catalytic steam reforming of methane an successive catalytic synthesis of the gas mixture obtained, without successive purification, such as removal of water and higher alcohols. The mixture formed is extremely suitable for dispersion in petrol by means of surface-active substances and optionally a higher alcohol, in which process a mixture is obtained which remains clear and stable within a wide temperature range (-20°C to +30°C). The mixture obtained contains, in respect of methanol, 10-25% by volume of water and 0.05-0.5% by volume or more of higher alcohols.

In order even further to improve the stability of the clear liquid mixture obtained even further, the mixture may additionally contain an ether with 2-8 C atoms, specifically methyl-tertiary butylether. The alcohol not soluble in water can then be partly replaced by the said ether. Preferably 0.01 to 15% by weight, specifically 0.05-10% by weight, of ether is added.

### Example I

Clear liquid mixtures were formed by bringing together in a test tube:
Premium petrol (RON=99; MON=88; boiling range 35 to 200°C); methanol in the form of crude methanol with 21.5% by volume of water and 0.02% by volume of alcohols not or sparingly soluble in water, such as butanol, pentanol and higher alcohols, and 0.08% by volume of alcohols completely soluble in water, such as ethanol and propanol; or pure methanol with 21.5% by volume of water; a mixture of Na-oleate and oleic acid in the ratio of 80:20 and n-butanol.

The mixture of surface-active substances was dissolved in the alcohol mixture and as such added to the petrol.

The quantities of the various components are mentioned in the following table, which also states if the mixture is stable after 1 day's storage at-20°C.

With 1.00 g methanol (pure and crude) the same results are obtained.

It is, furthermore, found that, if 0.75 to 1.75 g crude methanol is added, a clear mixture is obtained at both surfactant butanol ratios. It has, furthermore, been found that the stability range is twice as large as that when pure methanol with 21.5% by volume of water is used.

### Example II

In order to show the effects of different types of alcohol on the stability of the clear liquid mixture according to the invention, the quantities in grammes of each type of alcohol at +20°C respectively ―20°C to be added in order to obtain a clear stable liquid mixture were determined.

The mixture contains 10 ml regular petrol (RON 88; MON 82), 0.8 g ammonium oleate-oleic acid mixture in the proportion of 60:40; 1.8 g crude methanol of the composition as in example I.

These results show that the non-soluble alcohols, particularly n-butanol and n-pentanol, clearly produce the greatest effects.

### Example III

In this example the effect of the addition of methyl-tertiary-butylether (MTBE) on the stability of the liquid mixtures according to the invention is shown.

The results are given in the following table. A mixture of regular petrol, surfactants and crude methanol was started from as in example II.

## Claims

1. Clear liquid mixture for application as fuel in combustion engines, comprising:
a liquid hydrocarbon mixture;
water;
an alcohol fully soluble in water;
surface-active substances;
characterized in that the fuel mixture consists of:
a. a liquid hydrocarbon mixture;
b. a mixture of methanol, water and higher alcohols, that has been obtained by steam reforming of methane and subsequent catalytic synthesis of the gas mixture obtained, in such amount that the fuel mixture contains 1-10% by weight of water; 0,1-25% by weight of methanol and 0,01-20% by weight of alcohols with 4 to 12 C atoms not or sparingly soluble in water;
c. 0,1-15% by weight of surface-active substances; and optionally
d. 5-20% by weight of an alcohol with 2-12 C atoms, and/or
e. 0,01-15% by weight of an ether with 2-8 C atoms.

2. Clear liquid mixture according to claim 1, characterized in that the liquid mixture of methanol, water and higher alcohols is present in such an amount that the fuel mixture contains 1-10% by weight of water; 0,1-25% by weight of methanol; 0,01-20% by weight of alcohols with 4 to 12 C atoms not or sparingly soluble in water and 5-10% by weight of alcohols with 2-4 C atoms fully soluble in water.

3. Clear liquid mixture according to claim 1, characterized in that the mixture of methanol, water and higher alcohols is present in such an amount that the fuel mixture contains 1-10 by weight of water, 0,1-25% by weight of methanol, 5-20% by weight of alcohols with 4-12 C atoms not or sparingly soluble in water and 0,01-5% by weight of alcohols with 2-4 C atoms fully soluble in water.

4. Clear liquid mixture according to any one of claims 1-3, characterized in that the mixture of methanol water and higher alcohols is present in such an amount that the fuel mixture contains.1-5% by weight of water and 2-15% by weight of methanol.

## Patentansprüche

1. Klares, flüssiges Gemisch zur Verwendung als Kraftstoff in Verbrennungsmotoren, enthaltend:
ein flüssiges Kohlenwasserstoffgemisch,
Wasser,
einen völlig wasserlöslichen Alkohol,
oberflächenaktive Substanzen,
dadurch gekennzeichnet, daß das Kraftstoffgemisch aus:
a) einem flüssigen Kohlenwasserstoffgemisch,
b) einem Gemisch aus Methanol, Wasser und höheren Alkoholen, das durch Dampfreformieren von Methan und nachfolgende katalytische Synthese des erhaltenen Gasgemischs mit solchen Werten erzielt wird, daß das Kraftstoffgemisch 1 bis 10 Gew.-% Wasser, 0,1 bis 25 Gew.-% Methanol und 0,01 bis 20 Gew.-% nicht oder schwer wasserlösliche Alkohole mit 4 bis 12 C-Atomen enthält,
c) 0,1 bis 15 Gew.-% oberflächenaktiben Substanzen und wahlweise
d) 5 bis 20 Gew.-% eines Alkohols mit 2 bis 12 C-Atomen und/oder
e) 0,01 bis 15 Gew.-% eines Äthers mit 2 bis 8 C-Atomen
besteht.

2. Klares, flüssiges Gemisch nach Anspruch 1, dadurch gekennzeichnet, daß das flüssige Gemisch aus Methanol, Wasser und höheren Alkoholen in einem solchen Umfang vorliegt, daß das Kraftstoffgemisch 1 bis 10 Gew.-% Wasser, 0,1 bis 25 Gew.-% Methanol, 0,01 bis 20 Gew.-% nicht oder schwer wasserlösliche Alkohole mit 4 bis 12 C-Atomen und 5 bis 10 Gew.-% völlig wasserlösliche Alkohole mit 2 bis 4 C-Atomen enthält.

3. Klares, flüssiges Gemisch nach Anspruch 1, dadurch gekennzeichnet, daß das Gemisch aus Methanol, Wasser und höheren Alkoholen in einem solchen Umfang vorliegt, daß das Kraftstoffgemisch 1 bis 10 Gew.-% Wasser, 0,1 bis 25 Gew.-% Methanol, 5 bis 20 Gew.-% nicht oder schwer wasserlösliche Alkohole mit 4 bis 12 C-Atomen und 0,01 bis 5 Gew.-% völlig wasserlösliche Alkohole mit 2 bis 4 C-Atomen enthält.

4. Klares, flüssiges Gemisch nach einem der Ansprüche 1 bis 3, dadurch gekennzeichnet, daß das Gemisch aus Methanol, Wasser und höheren Alkoholen in solch einem Umfang vorliegt, daß das Kraftstoffgemisch 1 bis 5 Gew.-% Wasser und 2 bis 15 Gew.-% Methanol enthält.

## Revendications

1. Mélange liquide limpide pour des applications comme combustible dans les moteurs à combustion, comprenant:
un mélange liquide d'hydrocarbures;
de l'eau;
un alcool entièrement soluble dans l'eau;
des substances tensio-actives;
caractérisé en ce que le mélange combustible est constitué par:
a. un mélange liquide d'hydrocarbures;
b. un mélange de méthanol, d'eau et d'alcools supérieurs qui a été obtenu par reforming à la vapeur du méthane suivi d'une synthèse catalytique du mélange gazeux obtenu, en quantités telles que le mélange combustible contienne 1-10% en poids d'eau; 0,1-25% en poids de méthanol et 0,01 - 20% en poids d'alcools ayant 4 à 12 atomes de C pas ou peu solubles dans l'eau;
c. 0,1-15% en poids de substances tensio-actives; et, éventuellement,
d. 5-20% en poids d'un alcool à 2-12 atomes de C, et/ou
e. 0,01-15% en poids d'un éther à 2-8 atomes de C.

2. Mélange liquide limpide selon la revendication 1, caractérisé en ce que le mélange liquide de méthanol, d'eau et d'alcools supérieurs est présent en quantité telle que le mélange combustible contienne 1-10% en poids d'eau; 0,1-25% en poids de méthanol; 0,01-20% en poids d'alcools ayant 4 à 12 atomes de C pas ou peu solubles dans l'eau et 5-10% en poids d'alcools ayant 2-4 atomes de C entièrement solubles dans l'eau.

3. Mélange liquide limpide selon la revendication 1, caractérisé en ce que le mélange de méthanol, d'eau et d'alcools supérieurs est présent en quantité telle que le mélange combustible contienne 1-10% en poids d'eau, 0,1 -25% en poids de méthanol, 5-20% en poids d'alcools ayant 4-12 atomes de C pas ou peu solubles dans l'eau et 0,01-5% en poids d'alcools ayant 2-4 atomes de C entièrement solubles dans l'eau.

4. Mélange liquide limpide selon l'une quelconque des revendications 1 à 3, caractérisé en ce que le mélange de méthanol, d'eau et d'alcools supérieurs est présente en quantité telle que le mélange combustible contienne 1-5% en poids d'eau et 2-15% en poids de méthanol.
